









FIG. 2A



FIG. 2B



FIG. 3



FIG. 4A





FIG. 5A

FIG. 5B





FIG. 5C

SOFT MAGNETIC ALLOY AND MAGNETIC  
COMPONENT

## TECHNICAL FIELD

The present disclosure relates to a soft magnetic alloy, and a magnetic component using the soft magnetic alloy.

## BACKGROUND

As a magnetic material used for various magnetic components such as an inductor and the like, soft magnetic alloys shown in Patent Documents 1 to 3 are known. These soft magnetic alloys have a higher saturation magnetic flux density than a ferrite material, and exhibits good soft magnetic properties. Note that, occasionally, corrosion such as rust and the like may be formed to a soft magnetic alloy, thus an improved corrosion resistant of the soft magnetic alloy was demanded.

[Patent Document 1] Patent Application Laid Open No. 2009-293099

[Patent Document 2] Patent Application Laid Open No. 2007-231415

[Patent Document 3] Patent Application Laid Open No. 2014-167139

## SUMMARY

The present disclosure is achieved in view of such circumstances, and the object is to provide a soft magnetic alloy having a high corrosion resistance, and a magnetic component using the soft magnetic alloy.

In order to achieve the above object, a soft magnetic alloy according to the present disclosure includes

an internal area having a soft magnetic type alloy composition including Fe and Co,

a Co concentrated area existing closer to a surface side than the internal area and having a higher Co concentration than in the internal area, and

a SB concentrated area existing closer to the surface side than the Co concentrated area and having a higher concentration of at least one element selected from Si and B than in the internal area.

As a result of keen study by the present inventors, the soft magnetic alloy satisfying the above-described characteristics can suppress rust formation when it is immersed in water, thus a corrosion resistance is improved.

Preferably, the SB concentrated area may include an oxide phase. Also, preferably the SB concentrated area may include amorphous.

Preferably, the Co concentrated area may include a metal phase. Also, preferably, a Co concentration degree in the Co concentrated area may be larger than 1.2.

Preferably, an amorphous degree of the soft magnetic alloy may be 85% or higher.

The soft magnetic alloy may be in a form of ribbon or in a form of powder.

The use of the soft magnetic alloy of the present disclosure is not particularly limited, and for example, it can be used for various coil components such as an inductor and the like, a filter, and various magnetic components such as an antenna, and the like. Among the above-mentioned uses, the soft magnetic alloy of the present disclosure is suitable as a material for a magnetic core in the coil component and the like.

BRIEF DESCRIPTION OF THE SEVERAL  
VIEWS OF THE DRAWINGS

FIG. 1A is an enlarged cross section of an essential part 5 of a soft magnetic alloy 1 according to an embodiment of the present disclosure.

FIG. 1B is an example of an enlarged cross section of a soft magnetic alloy 1a according to an embodiment of the present disclosure.

10 FIG. 2A is an example of a chart obtained from an X-ray crystallography.

FIG. 2B is an example of a pattern obtained by profile fitting the chart shown in FIG. 2A.

15 FIG. 3 is an example of a graph obtained by performing a line analysis using EDX along a measurement line L<sub>M</sub> shown in FIG. 1A.

FIG. 4A is a cross section showing a soft magnetic alloy 1b according to an embodiment of the present disclosure.

20 FIG. 4B is an enlarged cross section of an area IVB shown in FIG. 4A.

FIG. 5A is an example of an EELS image of the soft magnetic alloy 1 shown in FIG. 1A.

FIG. 5B is an example of an EELS image of the soft magnetic alloy 1a shown in FIG. 1B.

25 FIG. 5C is an example of an STEM image of the soft magnetic alloy 1b shown in FIG. 4A.

## DETAILED DESCRIPTION

30 Hereinafter, the present disclosure is described in further detail based on embodiments shown in the figures.

A soft magnetic alloy 1 of the present embodiment can be a ribbon form, a powder form, a block form, and the like; and a shape of the soft magnetic alloy 1 is not particularly limited. Also, a size of the soft magnetic alloy 1 is not particularly limited. For example, when the soft magnetic alloy 1 is a ribbon form, a thickness of the ribbon may be within a range of 15  $\mu\text{m}$  to 100  $\mu\text{m}$ . When the soft magnetic alloy 1 is a powder form, an average particle size of the soft 35 magnetic alloy powder can be within a range of 0.5  $\mu\text{m}$  to 150  $\mu\text{m}$ , and preferably within a range of 0.5  $\mu\text{m}$  to 25  $\mu\text{m}$ .

40 Note that, the above-mentioned average particle size can be measured by using various particle size analyzing method such as a laser diffraction method and the like; and preferably, the average particle size may be measured by using a particle image analyzer Morphologi G3 (made by Malvern Panalytical Ltd). A Morphologi G3 is a device which disperses the soft magnetic alloy powder using air, and a projected area of the individual particle constituting the 45 powder is measured, then a particle size distribution of a circle equivalent diameter from the projected area is obtained. Then, from the obtained particle size distribution, the average particle size is a particle size where a volume-based or number-based cumulative relative frequency is 50 50%. Note that, when the soft magnetic alloy 1 is included in the magnetic core, the average particle size of the soft magnetic alloy 1 (powder) is obtained by measuring the circle equivalent diameter of the particle included in the cross section by observing the cross section using an electron microscope (SEM, STEM, and the like).

55 FIG. 1A is a cross section which is an enlarged image near a surface of the soft magnetic alloy 1. As shown in FIG. 1A, the soft magnetic alloy 1 includes an internal area 2, a Co concentrated area 11 is positioned closer to the surface side 60 of the soft magnetic alloy 1 than the internal area 2, and a SB concentrated area 12 is positioned closer to the surface side of the soft magnetic alloy 1 than the Co concentrated

area 11. Note that, in the present embodiment, "an inner side" means a side closer to a center of the soft magnetic alloy 1, "a surface side" or "an outer side" means a side away from the center of the soft magnetic alloy 1.

### Internal Area 2

The internal area 2 is a main part of the soft magnetic alloy 1 which occupies at least 90 vol % of a volume of the soft magnetic alloy 1. Thus, an average composition of the soft magnetic alloy 1 can be considered as a composition of the internal area 2; and a crystal structure of the soft magnetic alloy 1 can be considered as a crystal structure of the internal area 2. Note that, a volume ratio of the above-mentioned internal area 2 is interchangeable with an area ratio, and the internal area 2 occupies at least 90% of a cross section of the soft magnetic alloy 1.

The internal area 2 (that is, the soft magnetic alloy 1) has a soft magnetic type alloy composition including Fe and Co, and a specific alloy composition is not particularly limited. For example, the internal area 2 can be a crystal type soft magnetic alloy such as a Fe—Co based alloy, a Fe—Co—V based alloy, a Fe—Co—Si based alloy, a Fe—Co—Si—Al based alloy, and the like. Further, in the internal area 2, P is preferably included, and as a crystal type soft magnetic alloy including P, a Fe—Co—Si—P based alloy, a Fe—Co—Si—P—Cr based alloy, and the like may be mentioned. By including P in the internal area 2, Co tends to easily concentrate at an outer edge of the internal area 2.

Also, from the point of lowering a coercivity, the internal area 2 is preferably constituted by an amorphous alloy composition or a nanocrystal alloy composition. As an amorphous or nanocrystal soft magnetic alloy, a Fe—Co—P—C based alloy, a Fe—Co—B based alloy, a Fe—Co—B—Si based alloy, or the like may be mentioned. More specifically, the internal area 2 is preferably constituted by an alloy composition satisfying a compositional formula of  $(Fe_{1-(\alpha+\beta)}Co_{\alpha}Ni_{\beta})_{1-\gamma}X_{1-\gamma}(1-(a+b+c+d+e))B_aP_bSi_cC_dCr_e$ . As the internal area 2 is constituted by the alloy composition satisfying the above-compositional formula, a crystal structure made of amorphous, heteroamorphous, or nanocrystals tends to be obtained easily.

In the above-mentioned compositional formula, "B" is boron, "P" is phosphorous, "C" is carbon, and X1 is at least one selected from Ti, Zr, Hf, Nb, Ta, Mo, W, Al, Ga, Ag, Zn, S, Ca, Mg, V, Sn, As, Sb, Bi, N, O, Au, Cu, rare earth elements, and platinum group elements. The rare earth elements include Sc, Y, and lanthanoids; and the platinum group elements include Ru, Rh, Pd, Os, Ir, and Pt. Also,  $\alpha$ ,  $\beta$ ,  $\gamma$ ,  $a$ ,  $b$ ,  $c$ ,  $d$ , and  $e$  represent atomic ratios, and these atomic ratios preferably satisfy the following relations.

A Co amount ( $\alpha$ ) with respect to Fe may be within a range of  $0.005 \leq \alpha \leq 0.700$ , may be within a range of  $0.010 \leq \alpha \leq 0.600$ , may be within a range of  $0.030 \leq \alpha \leq 0.600$ , or may be within a range of  $0.050 \leq \alpha \leq 0.600$ . When the Co amount ( $\alpha$ ) is within the above-mentioned range, a saturation magnetic flux density (Bs) and the corrosion resistance improve. From the point of improving Bs, the Co amount ( $\alpha$ ) may preferably be within a range of  $0.050 \leq \alpha \leq 0.500$ . As the Co amount ( $\alpha$ ) increases, the corrosion resistance tends to improve; and when the Co amount ( $\alpha$ ) is too large, Bs tends to decrease easily.

Also, a Ni amount ( $\beta$ ) with respect to Fe may be within a range of  $0 \leq \beta \leq 0.200$ . That is, Ni may not be included, and the Ni amount ( $\beta$ ) may be within a range of  $0.005 \leq \beta \leq 0.200$ . From the point of improving Bs, the Ni amount ( $\beta$ ) may be within a range of  $0 \leq \beta \leq 0.050$ , may be within a of

$0.001 \leq \beta \leq 0.050$ , or may be within a range of  $0.005 \leq \beta \leq 0.010$ . As the Ni amount ( $\beta$ ) increases, the corrosion resistance tends to improve, and when the Ni amount ( $\beta$ ) is too large, Bs decreases.

5 X1 may be included impurities, or may be added intentionally. A X1 amount ( $\gamma$ ) may be within a range of  $0 \leq \gamma \leq 0.030$ . That is, less than 3.0% of a total amount of Fe, Co, and Ni may be substituted by X1.

Further, when a sum of atomic ratios of elements constituting the soft magnetic alloy is 1, an atomic ratio of a total amount of Fe, Co, Ni, and X1 is preferably within a range of  $0.720 \leq (1-(a+b+c+d+e)) \leq 0.950$ , and more preferably is within a range of  $0.780 \leq (1-(a+b+c+d+e)) \leq 0.890$ . When the above-mentioned relation is satisfied, Bs tends to improve easily. Also, when  $0.720 \leq (1-(a+b+c+d+e)) \leq 0.890$  is satisfied, an amorphous soft magnetic alloy is easily obtained.

The atomic ratio of B is represented by "a", and "a" is preferably within a range of  $0 \leq a \leq 0.200$ ; and from the point of improving Bs, "a" is more preferably within a range of  $0 \leq a \leq 0.150$ .

The atomic ratio of P is represented by "b", and "b" is preferably within a range of  $0 \leq b \leq 0.100$ . That is, P may not be included, and from the point of improving both Bs and the corrosion resistance, "b" is preferably within a range of  $0.001 \leq b \leq 0.100$ , more preferably within a range of  $0.005 \leq b \leq 0.080$ , and particularly preferably within a range of  $0.005 \leq b \leq 0.050$ .

The atomic ratio of Si is represented by "c", and "c" is preferably within a range of  $0 \leq c \leq 0.150$ . That is, Si may not be included; and from the point of improving both Bs and the corrosion resistance, "c" is more preferably within a range of  $0.001 \leq c \leq 0.070$ .

The atomic ratio of C is represented by "d", and "d" is preferably within a range of  $0 \leq d \leq 0.050$ . That is, C may not be included; and from the point of improving both Bs and the corrosion resistance, "d" is more preferably within a range of  $0 \leq d \leq 0.020$ .

The atomic ratio of Cr is represented by "e", and "e" is preferably within a range of  $0 \leq e \leq 0.050$ . That is, from the point of improving Bs, Cr may not be included; and from the point of improving both Bs and the corrosion resistance, "e" is more preferably within a range of  $0.001 \leq e \leq 0.020$ .

The composition of the above-mentioned internal area 2 (that is, the composition of the soft magnetic alloy 1) can be analyzed, for example, by using Inductively Coupled Plasma (ICP). Here, when it is difficult to determine an oxygen amount by using ICP, an impulse heat melting extraction method can be used. Also, if it is difficult to determine a carbon amount and a sulfur amount by using ICP, an infrared absorption method can be used.

Also, other than ICP, a compositional analysis may be carried out by EDX (Energy Dispersive X-ray Spectroscopy) or EPMA (Energy Probe Microanalyzer) using an electron microscope. For example, regarding the soft magnetic alloy 1 included in a magnetic core which includes a resin component, a compositional analysis using ICP may be difficult in some cases. In such case, the compositional analysis may be carried out using EDX or EPMA. Also, if a detailed compositional analysis is difficult by any of the above-mentioned methods, the detailed compositional analysis may be performed using 3DAP (three dimensional atom probe). In case of using 3DAP, the influence of the resin component, a surface oxidation, and the like are excluded from the area of analysis, then the composition of the soft magnetic alloy 1, that is the composition of the internal area 2, can be determined. This is because when

## 5

3DAP is used, a small area (for example, an area of  $\phi 20$  nm $\times$ 100 nm) is set in the soft magnetic alloy **1** to determine an average composition.

Note that, in case a line analysis of a cross section near the surface side of the soft magnetic alloy **1** is carried out by using EDX or EELS (Electron Energy Loss Spectroscopy), the internal area **2** can be recognized as an area having stable concentrations of Fe and Co (see FIG. 3). Also, for example, the average composition obtained by performing a mapping analysis to the internal area **2** can be considered as the composition of the soft magnetic alloy **1**. In such case, the mapping analysis is performed using EDX or EELS; and an area to be measured is an area which is 100 nm or more away in a depth direction from the surface of the soft magnetic alloy **1** (corresponds to the internal area **2**), and an area of measurement may be about 256 nm $\times$ 256 nm or so.

A crystal structure of the internal area **2** (that is, a crystal structure of the soft magnetic alloy **1**) can be a crystalline structure, a nanocrystal structure, or an amorphous structure; and preferably the crystal structure of the internal area **2** may be an amorphous structure. In other words, an amorphous degree X of the internal area **2** (that is, an amorphous degree X of the soft magnetic alloy **1**) may preferably be 85% or more. The crystal structure having the amorphous degree X of 85% or more is a structure which is mostly made of amorphous, or heteroamorphous. The structure made of heteroamorphous is a structure in which crystals slightly exist inside amorphous. That is, in the present embodiment, “a crystal structure is amorphous” means that a crystal structure has the amorphous degree X of 85% or more; and crystals may be included as long as the amorphous degree X satisfies the above-mentioned range.

Note that, in case the structure is heteroamorphous, the average crystal particle size of the crystals existing in amorphous structure may preferably be within a range of 0.1 nm or more and 10 nm or less. Also, in the present embodiment, “nanocrystal” refers to a structure in which the amorphous degree X is less than 85% and the average crystal particle size is 100 nm or less (preferably, 3 nm to 50 nm). Further, “crystalline” refers to a crystal structure in which the amorphous degree X is less than 85% and the average crystal particle size is larger than 100 nm.

The amorphous degree X can be measured by X-ray crystallography using XRD. Specifically,  $2\theta/\theta$  measurement is performed using XRD to the soft magnetic alloy **1** according to the present embodiment, and a chart shown in FIG. 2A is obtained. Here, a measurement range of a diffraction angle  $2\theta$  may preferably be set to a range in which amorphous-derived halos can be confirmed, for example within a range of  $2\theta=30^\circ$  to  $60^\circ$ .

Next, the chart shown in FIG. 2A is profile-fitted using a Lorentz function represented by the following equation (2). In this profile fitting, a difference between the integrated intensities actually measured by using XRD and the integrated intensities calculated using the Lorentz function is preferably within 1%. As a result of this profile fitting, as shown in FIG. 2B, a crystal component pattern  $\alpha_c$  which indicates a crystal scattering integrated intensity  $I_c$ , an amorphous component pattern  $\alpha_a$  which indicates an amorphous scattering integrated intensity  $I_a$ , and a pattern  $\alpha_{c+a}$  which is a combination of these two are obtained. Then, the crystal scattering integrated intensity  $I_c$  and the amorphous

## 6

scattering integrated intensity  $I_a$  are placed in the below equation (1), thereby the amorphous degree X is obtained.

$$X=100-(I_c/(I_c+I_a)\times 100) \quad \text{Equation (1)}$$

$I_c$ : Crystal scattering integrated intensity  
 $I_a$ : Amorphous scattering integrated intensity

[Formula 1]

$$f(x) = \frac{h}{1 + \frac{(x - u)^2}{w^2}} + b \quad \text{Equation 2}$$

h: Peak height  
u: Peak position  
w: Half bandwidth  
b: Background height

Note that, a method of measuring the amorphous degree X is not limited to a method using the above-mentioned XRD, and the amorphous degree X may be measured by using EBSD (Electron BackScatter Diffraction) or electron diffraction.

Co Concentrated Area **11**

The Co concentrated area **11** is an area having a higher concentration of Co than in the internal area **2**. In the present embodiment, this Co concentrated area **11** may preferably be an amorphous metal phase continuous from the internal area **2**, and covers at least part of a periphery of the internal area **2**. A coverage of the Co concentrated area **11** with respect to the internal area **2** in the cross section of the soft magnetic alloy **1** is not particularly limited, and the coverage can be 50% or more, or more preferably it is 80% or more.

The cross section of the surface area of the soft magnetic alloy **1** is observed using STEM (scanning transmission electron microscope) or TEM (transmission electron microscope), and at the same time a mapping analysis is performed using EDX or EELS, thereby the presence of the Co concentrated area **11** and the coverage thereof can be verified. For example, an image (EELS image) shown in FIG. 5A is an example of the mapping analysis result by EELS. The EELS image on the left side of FIG. 5A shows the Co distribution, and a shade of Co is expressed by a contrast of bright or dark. In said EELS image, the internal area **2** can be recognized as an area where almost no shade of Co can be seen in Co concentration distribution. Further, at the edge of the internal area **2** the contrast becomes brighter, and this implicates that the Co concentration is higher than in the internal area **2**. This area with a high Co concentration is the Co concentrated area **11**, and the presence of the Co concentrated area **11** can be confirmed by the EELS image of Co.

An average thickness  $t_1$  of the Co concentrated area **11** identified by this mapping analysis is preferably 0.3 nm or more. The upper limit of  $t_1$  is not particularly limited, and for example it can be 30.0 nm or less. When  $t_1$  is thickened within this preferable range, further enhanced corrosion resistance can be obtained. Note that, the average thickness  $t_1$  is preferably calculated by measuring the thickness of the Co concentrated area **11** at least from 3 different points by changing the area of measurement.

As mentioned in above, the Co concentrated area **11** may be extremely thin in some cases, thus in case of identifying the Co concentrated area **11**, a line analysis is preferably used together with the mapping analysis. FIG. 3 is a sche-

matic diagram showing an example of a line analysis result along a measurement line  $L_M$  shown in FIG. 1A; and a vertical axis is a detection intensity of each element (that is, the intensity of characteristic X-ray), and a horizontal axis is a distance (depth) from the outermost surface **10**. As shown in FIG. 3, the line analysis results show a high peak of Co concentration at the edge of the internal area **2** in which the concentrations of Fe and Co are stable. The area showing this peak of Co is the Co concentrated area **11**. In other words, a local maximum of the Co concentration exists in the Co concentrated area **11**, and due to the above-mentioned peak, the presence of the Co concentrated area **11** can be confirmed.

Also, the Co concentrated area **11** having said peak is a metal phase. A phase state of the Co concentrated area **11** can be verified for example by a line analysis, a mapping analysis, or analysis using EELS of STEM or TEM. Specifically, when the Co concentrated area **11** is a metal phase, a line analysis or a mapping analysis shows a lower oxygen concentration in the Co concentrated area **11** than an oxygen concentration in the SB concentrated area **12** (see FIG. 3). Also, when spectrums obtained by EELS are analyzed, ratios of oxides of Co and metal Co in the Co concentrated area **11** can be calculated. When a ratio of metal Co is larger than a ratio of oxides of Co, the Co concentrated area **11** is defined as a metal phase. Note that, in TEM image obtained by observation of the transmitted waves, the contrast of the Co concentrated area **11** is darker than the SB concentrated area **12** which is an oxide phase, hence this also enables to confirm that the Co concentrated area **11** is a metal phase.

Also, in the present embodiment, the Co concentration degree in the Co concentrated area **11** is defined by a ratio ( $C_{11Co}/C_{2Co}$ ) of a Co mole ratio in the Co concentrated area **11** ( $C_{11Co}$ ) with respect to a Co mole ratio in the internal area **2** ( $C_{2Co}$ ). The Co concentration degree is preferably larger than 1.02, and more preferably larger than 1.20. Note that, the upper limit of the Co concentration degree is not particularly limited, and for example it can be 20 or less.

When a soft magnetic alloy which is made of the internal area **2** without forming the Co concentrated area **11** is used as a standard alloy, the corrosion resistance of the soft magnetic alloy **1** of the present embodiment compared to the standard alloy tends to improve as the Co concentration degree increases. That is, the Co concentration degree and the corrosion resistance show a positive correlation. Note that, as the internal area **2** of the soft magnetic alloy **1** includes a predetermined amount of P, the Co concentration degree tends to increase easily, and the corrosion resistance tends to further improve.

$C_{2Co}$  and  $C_{11Co}$  used for the calculation of the Co concentration degree are measured by carrying out a component analysis using EELS. Specifically,  $C_{2Co}$  is a mole ratio of Co with respect to a total of Fe and Co detected in the internal area **2**, and  $C_{2Co}$  is calculated by analyzing the EELS spectrums. Similarly,  $C_{11Co}$  is a mole ratio of Co with respect to a total of Fe and Co detected in the Co concentrated area **11**. That is, the mole ratio of Co in each area is represented by "Co/(Fe+Co)". In order to remove the influence from the impurities (elements which are mixed while making the measurement sample), (Fe+Co) is used as a denominator. Note that, a resolution during said analysis is preferably set to 0.5 nm or less, and for measuring  $C_{2Co}$ , preferably a point which is a depth of 0.2  $\mu$ m or deeper from the outermost surface **10** of the soft magnetic alloy **1** towards the inside is measured. Also, the above-mentioned measure-

ment is performed to at least five observation fields, and the Co concentration degree is obtained as the average of the measurement results.

Note that, in the Co concentrated area **11**, Co is detected as a main constitution element, and other than this, elements which constitute the internal area **2** such as Fe and the like are also included in the Co concentrated area **11**. Further, in the Co concentrated area **11**, as similar to the concentration of Co, other elements may be concentrated as well; and as one of such other elements, P may be mentioned. In this case, in a mapping analysis and a line analysis, a highly concentrated area of P may be observed in a way which overlaps with a highly concentrated area of Co.

#### SB Concentrated Area **12**

The SB concentrated area **12** is an area having a higher concentration of at least one selected from Si and B than in the internal area **2**. In the SB concentrated area **12**, either one of Si or B may be concentrated, or both Si and B may be concentrated. In the present embodiment, this SB concentrated area **12** covers at least part of the periphery of the Co concentrated area **11**. Also, at a part where the Co concentrated area **11** does not exist, the SB concentrated area **12** may directly contact the internal area **2** and cover the internal area **2**. A coverage of the SB concentrated area **12** of the soft magnetic alloy **1** is not particularly limited, and for example it can be 50% or more, and preferably it can be 80% or more.

As similar to the Co concentrated area **11**, the presence of the SB concentrated area **12** can be verified by performing a mapping analysis using EDX or EELS. For example, an image on the right side of FIG. 5A showing an example of the analysis result is an EELS image showing a B distribution measured at the same point as the EELS image (Co-L) on the left side. The EELS image on the right side shows a shade of B in a brighter contrast, and the B concentration is confirmed to be higher at the surface side of the Co concentrated area **11** than in the internal area **2**. In case of FIG. 5A, this area with a high concentration of B is the SB concentrated area **12**.

An average thickness  $t_2$  of the SB concentrated area **12** identified by this mapping analysis is preferably 0.5 nm or more. The upper limit of  $t_2$  is not particularly limited, and for example it can be 30 nm or less. Note that, as similar to  $t_1$ , preferably, the thickness of the SB concentrated area **12** is measured at least from 3 different points by changing the areas of measurement, and the average thereof is calculated to determine the average thickness  $t_2$ .

Also, the SB concentrated area **12** is preferably identified by using both a mapping analysis and a line analysis. As shown in FIG. 3, according to a line analysis result, Si or/and B concentration peak (peak including the local maximum of Si or/and B) can be confirmed at a position closer to the surface side than the peak of Co; and the position where the peak of Si or/and B is found is the SB concentrated area **12**. Further specifically, the SB concentrated area **12** can be determined by a characteristic X-ray intensity derived from Si and B when a line analysis is carried out. That is, when the intensity of the SB concentrated area **12** is stronger than the intensity derived from Si and B of the internal area **2**, then it can be concluded that Si or/and B is concentrated. Note that, as mentioned in above, the amount of element can be mapped from the intensity of each element by carrying out a mapping analysis, hence the SB concentrated area **12** can be identified based on the obtained mapping image.

Regarding the SB concentrated area **12**, the concentration degrees of Si and B are represented by an intensity ratio, and this intensity ratio is calculated from a line analysis using EDX or EELS. Specifically, a detection intensity of Si in the SB concentrated area **12** is defined as  $C_{12_s}$ , a detection intensity of Si in the internal area **2** is defined as  $C_{2_s}$ , and a Si intensity ratio (concentration degree) in the SB concentrated area is defined as  $C_{12_s}/C_{2_s}$ . This Si intensity ratio is preferably measured using EDX from the point of a resolution, and when Si is concentrated in the SB concentrated area **12**, then the Si intensity ratio is larger than 1.0. In the present embodiment, preferably the Si intensity ratio is 1.1 or more, and more preferably it is 1.2 or more. Also, the upper limit of the Si intensity ratio is not particularly limited, and for example it can be 20 or less.

Similarly, a detection intensity of B in the SB concentrated area **12** is defined as  $C_{12_B}$ , a detection intensity of B in the internal area **2** is defined as  $C_{2_B}$ , and a B intensity ratio (concentration degree) in the SB concentrated area **12** is defined as  $C_{12_B}/C_{2_B}$ . This B intensity ratio is preferably measured using EELS from the point of a resolution, and when B is concentrated in the SB concentrated area **12**, then the B intensity ratio is larger than 1.0. In the present embodiment, preferably the B intensity ratio is 1.1 or more, and more preferably 1.2 or more. Also, the upper limit of the B intensity ratio is not particularly limited, and for example it can be 20 or less.

The SB concentrated area **12** is preferably an oxide phase. When the SB concentrated area **12** is an oxide phase, it can be confirmed that an area with a high concentration of oxygen which overlaps with the Si or/and B highly concentrated area. Also, in a line analysis result, the oxygen concentration is higher at the position where Si or/and B peak is found than in other areas (the internal area **2** and the Co concentrated area **11**). For example, FIG. 3 is an image showing that the peak of the Si concentration and the peak of the oxygen concentration overlap in the SB concentrated area **12**. Note that, when the SB concentrated area **12** is an oxide phase, in the TEM image, the SB concentrated area **12** can be recognized as an area having a brighter contrast than the internal area **2**. Also, regarding the SB concentrated area **12**, as similar to the Co concentrated area **11**, a phase state can be confirmed by analyzing the spectrums obtained from EELS.

Also, the SB concentrated area **12** is preferably amorphous. Here, a crystallinity of the SB concentrated area **12** is determined by the presence of a spot caused by a crystal in FFT (Fast Fourier Transformation) pattern. That is, if a spot is not found in FFT pattern of the SB concentrated area **12**, the SB concentrated area **12** is considered amorphous, and if a spot is found, then it is considered that the SB concentrated area is crystalline. This FFT pattern is obtained by observing the cross section including the SB concentrated area **12** using HRTEM (High Resolution Transmission Electron Microscope), then performing a Fast Fourier Transformation process to the obtained HRTEM image.

Alternatively, the crystallinity of the SB concentrated area **12** can be identified by image analyzing the HRTEM image. In the HRTEM image, due to a phase contrast, a regularly arranged lattice can be confirmed in a crystalline part, and a random pattern can be confirmed in an amorphous part. Thus, by analyzing the HRTEM image, an area  $S_{SB}$  of the SB concentrated area **12**, and an area  $S_{SB}^{amo}$  of the area with irregular pattern (that is, the amorphous part) included in the area of measurement are measured; then an area ratio of amorphous part can be calculated as a ratio of  $S_{SB}^{amo}$  to  $S_{SB}$ . In the present embodiment, the area ratio of the amorphous

part in the SB concentrated area **12** is preferably 85% or more, and when said condition is satisfied, then it is considered that the SB concentrated area **12** is amorphous.

Note that, the above-mentioned evaluation of the crystallinity can be carried out by a selected area method in a micro area, or by a nanodiffraction method.

Note that, in the SB concentrated area **12**, as mentioned in above, Si, B, and O are detected; and other than these, the constitution elements of the internal area **2** such as Fe, Co, and the like can be detected.

As discussed in above, the soft magnetic alloy **1** has a characteristic surface structure which includes the Co concentrated area **11** and the SB concentrated area **12**. Particularly, in the present embodiment, as shown in FIG. 1A, the SB concentrated area **12** is positioned at the outermost surface side, and constitutes the outermost surface **10**. Note that, other surface structure may exist at further outside of the SB concentrated area **12**.

For example, as the soft magnetic alloy **1a** of FIG. 1B shows, an oxide layer **13** including Fe may be formed so that it covers the surface side of the SB concentrated area **12**. In this case, the outermost surface **10** of the soft magnetic alloy **1a** is constituted by the oxide layer **13**. FIG. 5B is in fact an example of an EELS image of the soft magnetic alloy **1a** shown in FIG. 1B. As shown in FIG. 5B, an area having a higher concentration of Fe can be confirmed at a position closer to the surface side than the SB concentrated area **12**. That is, the Fe concentration is higher in the oxide layer **13** than in the Co concentrated area **11** and the SB concentrated area **12**. Furthermore, the oxide layer **13** preferably has a higher crystallized area ratio than the SB concentrated area **12**. The oxide layer **13** satisfying such characteristics may be formed together with the Co concentrated area **11** and the SB concentrated area **12** when these two areas (**11** and **12**) are being formed. An average thickness  $t_3$  of the oxide layer **13** is preferably 1 nm or more. The upper limit of  $t_3$  is not particularly limited, and for example it can be 30 nm or less.

Also, as the soft magnetic alloy **1b** of FIG. 4A and FIG. 4B shows, a coating layer **20** for insulation may be formed at the outside of the SB concentrated area **12** or at the outside of the oxide layer **13**. In this case, the outermost surface **10** of the soft magnetic alloy **1b** is constituted by the coating layer **20**. FIG. 5C is in fact an example of a STEM image of the soft magnetic alloy **1b** shown in FIG. 4A. In this STEM image, an area with brighter contrast can be verified at the outermost surface of the soft magnetic alloy **1b**, and this area is the coating layer **20**. This coating layer **20** is a coating layer which is formed by carrying out a surface treatment such as coating or so after the Co concentrated area **11** and the SB concentrated area **12** are formed. An average thickness of the coating layer **20** is preferably within a range of 5 nm or more and 100 nm or less, and more preferably it is 50 nm or less. Note that, as shown in FIG. 4A, in many cases, such coating layer **20** is formed to the soft magnetic alloy of a powder form, but the coating layer **20** may be formed to the soft magnetic alloy of a ribbon form.

As discussed in above, the surface structure of the soft magnetic alloy **1** can include other layers (such as the oxide layer **13** and the coating layer **20**) besides the Co concentrated area **11** and the SB concentrated area **12**. Even in case of having said other layers, the Co concentrated area **11** exist at the side which is in contact with the internal area **2**. Further, a perpendicular distance  $d_1$  from the outermost surface **10** to the Co concentrated area **11** is preferably 200 nm or less, more preferably 100 nm or less, and even more preferably 50 nm or less. Particularly in case that the coating layer **20** does not exist and the outermost surface **10** is

## 11

constituted by the oxide layer **13** or by the SB concentrated area **12**, the perpendicular distance **d1** is preferably 30 nm or less, and more preferably 20 nm or less.

Note that, a measurement sample for analyzing the Co concentrated area **11** and the SB concentrated area **12** is preferably produced by using a micro-sampling method which uses FIB (Focused Ion Beam). For example, a Pt film of a thickness of 30 nm or so is formed by spattering to the outermost surface **10** of the soft magnetic alloy **1** to protect the surface while processing, then using FIB, an area at a depth of about 2  $\mu$ m from the outermost surface is cut out, thereby a thin sample is obtained. Then, this thin sample is processed and thinned so that a thickness in a direction perpendicular to the depth direction is 20 nm or less. This sample formed into a thin film may be used as a measurement sample for TEM and HRTEM observation.

Hereinbelow, a method of producing the soft magnetic alloy **1** according to the present embodiment is described.

The main part (internal area **2**) of the soft magnetic alloy **1** can be produced by various melting methods, and preferably it may be made by using a method in which a molten is quenched. This is because the amorphous soft magnetic alloy **1** can be easily obtained by quenching. For example, the soft magnetic alloy **1** of a ribbon form can be produced by a single roll method, and the soft magnetic alloy **1** of a powder form can be produced by an atomization method. Hereinbelow, a method of obtaining a soft magnetic alloy ribbon formed by a single roll method, and a method of obtaining a soft magnetic alloy powder formed by a gas atomization method are described.

In a single roll method, raw materials (pure metal and the like) of elements constituting the soft magnetic alloy **1** are prepared and weighed so to satisfy the target alloy composition. Then, the raw materials of the elements are melted to produce a mother alloy. A method of melting for producing the mother alloy is not particularly limited, and for example a method of melting by using high frequency heating in a chamber at a predetermined degree of vacuum may be mentioned.

Next, the above-mentioned mother alloy is heated and melted to obtain a molten. A temperature of the molten may be determined by taking the melting point of the target alloy composition into consideration. For example, the temperature of the molten may be within a range of 1200° C. to 1600° C. In a single roll method, this molten is supplied using a nozzle and the like to a cooled rotating roll, thereby a soft magnetic alloy ribbon is produced along the rotating direction of the roll. A thickness of the ribbon can be regulated by adjusting a rotation speed of the roll, a distance between the nozzle and the roll, a temperature of the molten, and the like. Also, the temperature and the rotation speed of the roll may be set to a condition so that the amorphous soft magnetic alloy can be easily obtained. For example, the temperature of the roll is preferably within a range of 20° C. to 30° C., and a rotation speed is preferably within a range of 20 to 30 m/sec. Note that, an atmosphere inside the chamber is not particularly limited, and for example it can be air atmosphere or an inert gas atmosphere.

In a gas atomization method, as similar to the above-mentioned single roll method, a molten within a range of 1200° C. to 1600° C. is obtained, then the molten is sprayed in the chamber to produce a powder. Specifically, the molten is exhausted from an exhaust port towards a cooling part, and a high-pressured gas is sprayed to exhausted molten metal drops. By spraying the high-pressured gas to the molten metal drops, the molten metal drops scatter at the inside of the chamber, and as these collide against the

## 12

cooling part (cooling water), the molten metal drops cool solidify and form the soft magnetic alloy powder.

As the high-pressured gas, an inert gas such as nitrogen gas, argon gas, helium gas, and the like; or a reducing gas such as ammonium decomposition gas and the like is preferably used. A spraying pressure of the high-pressured gas is preferably within a range of 2.0 MPa or more and 10 MPa or less. Also, a spraying amount of the exhausted molten is preferably within a range of 0.5 kg/min or more and 4.0 kg/min or less. In said gas atomization method, the particle size and the shape of the soft magnetic alloy powder can be adjusted by a ratio of a pressure of the high-pressured gas with respect to the spraying amount of the molten. The particle shape of the soft magnetic alloy powder obtained by this atomization method is usually a spherical shape, and an average circularity of the soft magnetic alloy powder is preferably 0.8 or more, more preferably 0.9 or more, and even more preferably 0.95 or more.

After obtaining the soft magnetic alloy of a ribbon form or a powder form as discussed in above, this soft magnetic alloy is heat treated at a low temperature in a predetermined oxygen concentration atmosphere under a predetermined pressure, thereby the Co concentrated area **11** and the SB concentrated area **12** are formed.

Specifically, a holding temperature during the heat treatment is preferably a temperature which does not crystallize the soft magnetic alloy, and for example it is preferably within a range of 200° C. to 400° C., and more preferably within a range of 200° C. to 300° C. Also, a temperature holding time is preferably within a range of 0.5 hours to 3.0 hours. An oxygen concentration inside a heating furnace is preferably within a range of 20 ppm or more and 2000 ppm or less, and more preferably within a range of 100 ppm or more and 1000 ppm or less. Further, while controlling the oxygen concentration inside the heating furnace as mentioned in above, an inert gas such as argon gas, nitrogen gas, or the like is introduced into the heating furnace so that the inside of the heating furnace has a positive pressure. A gauge pressure inside the heating furnace is preferably within a range of 0.05 kPa or more and 0.50 kPa or less, and more preferably within a range of 0.15 kPa or more and 0.45 kPa or less. Note that, a gauge pressure refers to a pressure of which atmospheric pressure is subtracted from an absolute pressure (a pressure when an absolute vacuum is 0 Pa).

By heat treating under such condition, the Co concentrated area **11** and the SB concentrated area **12** each having predetermined characteristics are formed to the surface side of the soft magnetic alloy. Also, depending on the conditions of the heat treatment, the oxide layer **13** including Fe may be formed at a surface side of the SB concentrated area **12**. Note that, when the soft magnetic alloy **1** is crystalline or nanocrystal (that is, when the amorphous degree X is less than 85%), a pre-heat treatment in order to control the crystallinity may be performed prior to the heat treatment for forming the above-mentioned concentrated areas.

In case of forming the coating layer **20** as shown in FIG. 4A and FIG. 4B, a coating treatment such as a phosphate coating treatment, a mechanical alloying treatment, a silane coupling treatment, a hydrothermal synthesis, and the like may be performed. As a type of coating layer **20** to be formed, phosphates, silicates, soda-lime glass, borosilicate glass, lead glass, aluminosilicate glass, borate glass, sulfate glass, and the like may be mentioned. Note that, as phosphates, for example, magnesium phosphate, calcium phosphate, zinc phosphate, manganese phosphate, cadmium phosphate, and the like may be mentioned. As silicates, sodium silicate and the like may be mentioned. When the

## 13

coating layer **20** is formed, improvements of the voltage resistance and the like can be expected in the magnetic core including the soft magnetic alloy **1**.

The soft magnetic alloy **1** including the Co concentrated area **11** and the SB concentrated area **12** is obtained by going through the above-mentioned steps. The soft magnetic alloy **1** of the present embodiment can be applied to various magnetic components, for example, a coil component such as an inductor, a filter, an antenna, and the like may be mentioned. Particularly, the soft magnetic alloy **1** according to the present embodiment is preferably applied to a magnetic core in a coil component such as an inductor. Note that, the soft magnetic alloy **1** may be constituted by mixing particle groups with different alloy compositions and particle sizes, and other magnetic materials which do not include concentrated areas **11** and **12** may be used together. For example, in the magnetic core including the soft magnetic alloy **1**, the magnetic materials not including the concentrated areas **11** and **12** may be included, and also other resin components may also be included.

## Summarizing the Present Embodiment

In the soft magnetic alloy **1** of the present embodiment, the Co concentrated area **11** and the SB concentrated area **12** each satisfying predetermined characteristics are formed to the outer side of the internal area **2** having a soft magnetic type alloy composition which includes Fe and Co. By having such characteristics, rust formation is suppressed when the soft magnetic alloy **1** is immersed in water, and the corrosion resistance can be improved. Particularly, when the Co concentrated area **11** has the Co concentration degree of larger than 1.20, the corrosion resistance of the soft magnetic alloy **1** can be further improved.

Also, by forming the Co concentrated area **11** and the SB concentrated area **12** to the amorphous soft magnetic alloy **1** having the amorphous degree of 85% or more, the corrosion resistance of the soft magnetic alloy **1** can be further improved while ensuring a high saturation magnetic flux density  $B_s$ .

Hereinabove, the embodiment of the present disclosure is described, however, the present disclosure is not limited to the above-mentioned embodiment, and it may be variously modified within the scope of the present disclosure.

## EXAMPLES

Hereinbelow, the present disclosure is described in further detail based on specific examples. Note that, the present disclosure is not limited to the examples. In tables shown in below, “\*\*” mark indicates a sample of comparative example.

## Experiment 1

In Experiment 1, a soft magnetic alloy powder was produced by using a gas atomization method. In a gas atomization method, the soft magnetic alloy powder of which a volume-based average particle size (D50) was within a range of 15 to 30  $\mu\text{m}$  was obtained under the conditions of a spraying temperature of a molten: 1500°C., a spraying amount of the molten: 1.2 kg/min, a pressure of a high-pressured gas: 7.0 MPa, and a water pressure of a cooling water: 10 MPa. Then, the soft magnetic alloy powder was heat treated under the conditions shown in Table 1, and soft magnetic alloys of Sample No. 2 to 11 were obtained. Also, in Experiment 1, a soft magnetic alloy of

## 14

Sample No. 1 which was not heat treated was also produced. Using this Sample No. 1 as a standard, evaluations shown in below were carried out.

## 5 Crystal Structure and Composition of the Soft Magnetic Alloy Powder

The composition of the soft magnetic alloy powder obtained by using a gas atomization method was measured using ICP. As a result, in all samples of Experiment 1, the soft magnetic alloy powder (that is the internal area **2**) of each sample was confirmed to have an alloy composition satisfying a compositional formula:  $(\text{Fe}_{0.7}\text{Co}_{0.3})_{0.84}\text{B}_{0.11}\text{Si}_{0.03}\text{C}_{0.01}\text{Cr}_{0.01}$  (atomic ratio;  $\alpha=0.300$ ,  $\beta=0$ ,  $\gamma=0$ ,  $a=0.110$ ,  $b=0$ ,  $c=0.030$ ,  $d=0.010$ , and  $e=0.010$ ). Also, when the soft magnetic alloy powders of Experiment 1 were performed with X-ray crystallography using XRD, each sample of Experiment 1 showed that the soft magnetic alloy powder (that is the internal area **2**) was amorphous satisfying 85% or more of an amorphous degree.

## Analysis of Surface Structure

From the soft magnetic alloy of each sample of Experiment 1, a thin sample near the surface was taken by a micro sampling method using FIB. Further, using the thin sample, a mapping analysis was carried out using TEM-EDX to examine the Co concentrated area **11** and the SB concentrated area **12**. Further, a component analysis of a specific area was carried out using TEM-EELS, and a Co concentration degree of the Co concentrated area **11** was measured. Analysis results of each sample of Experiment 1 are shown in Table 1. Note that, for the samples which were confirmed with the Co concentrated area **11** and the SB concentrated area **12**, an observation using HRTEM was carried out, and a phase state of each area was verified. As a result, in the samples having the Co concentrated area **11** (that is, Sample No. 3 to 8, 10, and 11) of Experiment 1, it was confirmed that the Co concentrated area **11** was an amorphous metal phase, and the SB concentrated area **12** was an amorphous oxide phase.

Saturation Magnetic Flux Density  $B_s$ 

45 The saturation magnetic flux density  $B_s$  of each sample was measured using a vibrating sample magnetometer (VSM) under the condition of 1000 kA/m magnetic field. Results are shown in Table 1. When this  $B_s$  was 1.50 T or more it was considered good, and 1.70 T or more was considered even better.

## Immersion Test

First, before performing the immersion test, a magnetic 55 core sample was produced using the soft magnetic alloy of each sample. The magnetic core sample was produced by going through below described steps. Granules were obtained by mixing 3 parts by mass of an epoxy resin to 100 parts by mass of the soft magnetic alloy. Then, the granules were filled into a mold, and then pressure molded at a pressure of 4 ton/cm<sup>2</sup>, thereby a magnetic core sample of a toroidal shape having a size of an outer diameter of 11 mmφ, an inner diameter of 6.5 mmφ, and a height of 1.0 mm was obtained.

60 The immersion test was performed in order to evaluate the corrosion resistance of the magnetic core sample obtained in the above. For the immersion test, the magnetic core sample

was immersed in tap water, then a time which took to confirm rust formation by visual observation was measured (rust formation time). In Experiment 1, the corrosion resistance of each sample was evaluated with respect to a rust formation time  $T_1$  of the Sample No. 1. Specifically, in Experiment 1, when a rust formation time of a sample was 1.0 times or less than  $T_1$  (the rust formation time of Sample No. 1), then it was evaluated as "NG (Not Good)"; when a rust formation time of a sample was more than 1.0 times and less than 1.2 times of  $T_1$ , then it was evaluated as "G (Good)"; and when a rust formation time of a sample was 1.2 times or more than  $T_1$ , it was evaluated as "VG (very good)". Results of the immersion test evaluated by the above-mentioned "NG, G, and VG" are shown in Table 1.

TABLE 1

| Sample No. | Heat treatment condition |                |                          |                    | Analysis results of surface structure |                             | Saturation magnetic flux       |              |                           |
|------------|--------------------------|----------------|--------------------------|--------------------|---------------------------------------|-----------------------------|--------------------------------|--------------|---------------------------|
|            | Holding Temp. °C.        | Holding Time h | Oxygen concentration ppm | Gauge pressure kPa | Co concentrated area                  |                             | SB concentrated area Formation | density Bs T | Immersion test Evaluation |
|            |                          |                |                          |                    | Formation                             | Co concentration degree (-) |                                |              |                           |
| 1X         | —                        | —              | —                        | —                  | None                                  | —                           | Formed                         | 1.73         | Standard                  |
| 2X         | 200                      | 1.0            | 100                      | 0.00               | None                                  | —                           | Formed                         | 1.73         | NG                        |
| 3          | 200                      | 1.0            | 100                      | 0.05               | Formed                                | 1.02                        | Formed                         | 1.75         | G                         |
| 4          | 200                      | 1.0            | 100                      | 0.15               | Formed                                | 1.08                        | Formed                         | 1.75         | G                         |
| 5          | 200                      | 1.0            | 100                      | 0.30               | Formed                                | 1.91                        | Formed                         | 1.75         | VG                        |
| 6          | 200                      | 1.0            | 100                      | 0.45               | Formed                                | 2.02                        | Formed                         | 1.75         | VG                        |
| 7          | 200                      | 0.5            | 100                      | 0.15               | Formed                                | 1.06                        | Formed                         | 1.75         | G                         |
| 8          | 200                      | 3.0            | 100                      | 0.15               | Formed                                | 1.21                        | Formed                         | 1.75         | VG                        |
| 9X         | 200                      | 1.0            | 0                        | 0.15               | None                                  | —                           | Formed                         | 1.75         | NG                        |
| 10         | 200                      | 1.0            | 500                      | 0.15               | Formed                                | 2.01                        | Formed                         | 1.74         | VG                        |
| 11         | 200                      | 1.0            | 1000                     | 0.15               | Formed                                | 2.23                        | Formed                         | 1.73         | VG                        |

As shown in Table 1, in Sample No. 3 to 8, 10, and 11 which were heat treated at predetermined conditions, the Co concentrated area **11** and the SB concentrated area **12** were formed. Furthermore, for these samples, a good relative corrosion resistance was attained compared to a standard alloy (Sample No. 1 of which the heat treatment was not performed) while a high  $B_s$  was maintained. Note that, in Sample No. 3 to 8, 10, and 11, it was confirmed that a perpendicular distance  $d_1$  which was a distance from the outermost surface **10** to the Co concentrated area **11** was 30 nm or less. According to this result, it was proven that the corrosion resistance improved by forming the Co concentrated area **11** and the SB concentrated area **12** which satisfied the predetermined characteristics at a surface side of the soft magnetic alloy.

Also, according to the results shown in Table 1, it was confirmed that the Co concentration degree of the Co concentrated area **11** was preferably larger than 1.02, and more preferably larger than 1.2.

#### Experiment 2

In Experiment 2, the soft magnetic alloys of Sample No. 12 to 101 were obtained by changing the alloy compositions. The alloy composition of each sample was analyzed using ICP, and the results are shown in Table 2 to Table 7 (evaluation results of Experiment 1 are partially included).

Specifically, for Sample No. 12 to 25 shown in Table 2, each sample satisfied a compositional formula:  $(Fe_{1-\alpha}Co_{\alpha})_{0.84}B_{0.11}Si_{0.03}C_{0.01}Cr_{0.01}$  (atomic ratio;  $\beta=0$ ,  $\gamma=0$ ,  $a=0.110$ ,  $b=0$ ,  $c=0.030$ ,  $d=0.010$ , and  $e=0.010$ ), and a Co atomic ratio  $\alpha$  was varied, thereby the soft magnetic alloy was produced.

Note that, Sample No. 18 is the same sample as Sample No. 1, and Sample No. 19 is the same sample as Sample No. 5.

Also, for the soft magnetic alloys of Sample No. 26 to 45 shown in Table 3, the atomic ratios of Co, Ni, and X1 were respectively fixed to  $\alpha=0.30$ ,  $\beta=0$ , and  $\gamma=0$ ; and then the atomic ratios of metalloids (B, P, Si, and C) and Cr were varied.

Also, for Sample No. 46 to 49 shown in Table 4, each sample satisfied a compositional formula:  $(Fe_{1-(0.3+\beta)}Co_{0.3}Ni_{\beta})_{0.84}B_{0.11}Si_{0.03}C_{0.01}Cr_{0.01}$  (atomic ratios:  $\alpha=0.300$ ,  $\gamma=0$ ,  $a=0.110$ ,  $b=0$ ,  $c=0.030$ ,  $d=0.010$ , and  $e=0.010$ ), and a Ni atomic ratio  $\beta$  was varied, thereby the soft magnetic alloy was produced.

Also, for Sample No. 50 to 101 shown in Table 5 to Table 7, each sample satisfied a compositional formula:  $((Fe_{0.7}Co_{0.3})_{0.975}X1_{0.025})_{0.84}B_{0.11}Si_{0.03}C_{0.01}Cr_{0.01}$  (atomic ratios;  $\alpha=0.300$ ,  $\beta=0$ ,  $\gamma=0.025$ ,  $a=0.110$ ,  $b=0$ ,  $c=0.030$ ,  $d=0.010$ , and  $e=0.010$ ), and a type of X1 element was varied, thereby the soft magnetic alloy was produced.

Note that, all of the soft magnetic alloys of Experiment 2 had an amorphous degree X of 85% or more. Also, in Experiment 2, for each alloy composition, a sample performed with a predetermined heat treatment and a sample without the predetermined heat treatment were formed; and in Table 2 to Table 7, the sample performed with the heat treatment was shown as "Y", and the sample without the heat treatment was shown as "N". Also, conditions of the heat treatment of Experiment 2 were a holding temperature: 200°C., a holding time: 1 h, an oxygen concentration in a heating furnace: 100 ppm, and a gauge pressure in the heating furnace: 0.3 kPa.

Also, for each of Sample No. 12 to 101 of Experiment 2, as similar to Experiment 1,  $B_s$  was measured and the immersion test was performed. In the immersion test of Experiment 2, for the same composition, the rust formation time of a sample without the heat treat was defined as  $T_N$ , and the rust formation time of a sample performed with the heat treatment was defined as  $T_Y$ , then a sample which showed  $T_Y/T_N \leq 1.0$  was evaluated as "NG (Not Good)", a sample which showed  $1.0 < T_Y/T_N < 1.2$  was evaluated as "G (Good)", and a sample which showed  $1.2 \leq T_Y/T_N$  was evaluated as "VG (Very Good)". Evaluation results are shown in Table 2 to Table 7.

TABLE 2

| Sample No. | Alloy composition:                                                |                |                |                 |                |                 | Analysis results of surface structure |                      |                          | Saturation magnetic flux |      |                 |
|------------|-------------------------------------------------------------------|----------------|----------------|-----------------|----------------|-----------------|---------------------------------------|----------------------|--------------------------|--------------------------|------|-----------------|
|            | $(Fe_{(1-\alpha)}Co_{\alpha})_{(1-(a+b+c+d+e))}B_aP_bSi_cC_dCr_e$ |                |                |                 |                |                 | Heat                                  | Co concentrated area |                          | SB                       | flux |                 |
|            | $(\beta = 0, \gamma = 0)$                                         |                |                | treated         |                |                 |                                       | Co                   | concentrated             |                          |      |                 |
|            | Co <sub>α</sub>                                                   | B <sub>a</sub> | P <sub>b</sub> | Si <sub>c</sub> | C <sub>d</sub> | Cr <sub>e</sub> | or not Y or N                         | Formation            | concentration degree (-) | area Formation           | Bs T | test Evaluation |
| 12X        | 0.05                                                              | 0.11           | 0              | 0.03            | 0.01           | 0.01            | N                                     | None                 | —                        | Formed                   | 1.68 | Standard        |
| 13         | 0.05                                                              | 0.11           | 0              | 0.03            | 0.01           | 0.01            | Y                                     | Formed               | 3.67                     | Formed                   | 1.71 | VG              |
| 14X        | 0.10                                                              | 0.11           | 0              | 0.03            | 0.01           | 0.01            | N                                     | None                 | —                        | Formed                   | 1.69 | Standard        |
| 15         | 0.10                                                              | 0.11           | 0              | 0.03            | 0.01           | 0.01            | Y                                     | Formed               | 5.52                     | Formed                   | 1.71 | VG              |
| 16X        | 0.15                                                              | 0.11           | 0              | 0.03            | 0.01           | 0.01            | N                                     | None                 | —                        | Formed                   | 1.69 | Standard        |
| 17         | 0.15                                                              | 0.11           | 0              | 0.03            | 0.01           | 0.01            | Y                                     | Formed               | 3.86                     | Formed                   | 1.71 | VG              |
| 18X (1)    | 0.30                                                              | 0.11           | 0              | 0.03            | 0.01           | 0.01            | N                                     | None                 | —                        | Formed                   | 1.73 | Standard        |
| 19 (5)     | 0.30                                                              | 0.11           | 0              | 0.03            | 0.01           | 0.01            | Y                                     | Formed               | 1.91                     | Formed                   | 1.75 | VG              |
| 20X        | 0.50                                                              | 0.11           | 0              | 0.03            | 0.01           | 0.01            | N                                     | None                 | —                        | Formed                   | 1.63 | Standard        |
| 21         | 0.50                                                              | 0.11           | 0              | 0.03            | 0.01           | 0.01            | Y                                     | Formed               | 1.82                     | Formed                   | 1.65 | VG              |
| 22X        | 0.60                                                              | 0.11           | 0              | 0.03            | 0.01           | 0.01            | N                                     | None                 | —                        | Formed                   | 1.59 | Standard        |
| 23         | 0.60                                                              | 0.11           | 0              | 0.03            | 0.01           | 0.01            | Y                                     | Formed               | 1.66                     | Formed                   | 1.62 | VG              |
| 24X        | 0.70                                                              | 0.11           | 0              | 0.03            | 0.01           | 0.01            | N                                     | None                 | —                        | Formed                   | 1.53 | Standard        |
| 25         | 0.70                                                              | 0.11           | 0              | 0.03            | 0.01           | 0.01            | Y                                     | Formed               | 1.60                     | Formed                   | 1.55 | VG              |

TABLE 3

| Sample No. | Alloy composition:                                                |                |                |                 |                |                 | Analysis results of surface structure |                      |                          | Saturation magnetic flux |      |                 |
|------------|-------------------------------------------------------------------|----------------|----------------|-----------------|----------------|-----------------|---------------------------------------|----------------------|--------------------------|--------------------------|------|-----------------|
|            | $(Fe_{(1-\alpha)}Co_{\alpha})_{(1-(a+b+c+d+e))}B_aP_bSi_cC_dCr_e$ |                |                |                 |                |                 | Heat                                  | Co concentrated area |                          | SB                       | flux |                 |
|            | $(\beta = 0, \gamma = 0)$                                         |                |                | treated         |                |                 |                                       | Co                   | concentrated             |                          |      |                 |
|            | Co <sub>α</sub>                                                   | B <sub>a</sub> | P <sub>b</sub> | Si <sub>c</sub> | C <sub>d</sub> | Cr <sub>e</sub> | or not Y or N                         | Formation            | concentration degree (-) | area Formation           | Bs T | test Evaluation |
| 26X        | 0.300                                                             | 0.020          | 0.040          | 0.030           | 0.010          | 0.010           | N                                     | None                 | —                        | Formed                   | 1.78 | Standard        |
| 27         | 0.300                                                             | 0.020          | 0.040          | 0.030           | 0.010          | 0.010           | Y                                     | Formed               | 2.15                     | Formed                   | 1.80 | VG              |
| 28X        | 0.300                                                             | 0.200          | 0.000          | 0.000           | 0.000          | 0.010           | N                                     | None                 | —                        | Formed                   | 1.52 | Standard        |
| 29         | 0.300                                                             | 0.200          | 0.000          | 0.000           | 0.000          | 0.010           | Y                                     | Formed               | 2.31                     | Formed                   | 1.55 | VG              |
| 30X        | 0.300                                                             | 0.110          | 0.030          | 0.030           | 0.010          | 0.010           | N                                     | None                 | —                        | Formed                   | 1.67 | Standard        |
| 31         | 0.300                                                             | 0.110          | 0.030          | 0.030           | 0.010          | 0.010           | Y                                     | Formed               | 2.23                     | Formed                   | 1.70 | VG              |
| 32X        | 0.300                                                             | 0.110          | 0.070          | 0.030           | 0.010          | 0.010           | N                                     | None                 | —                        | Formed                   | 1.53 | Standard        |
| 33         | 0.300                                                             | 0.110          | 0.070          | 0.030           | 0.010          | 0.010           | Y                                     | Formed               | 2.42                     | Formed                   | 1.55 | VG              |
| 34X        | 0.300                                                             | 0.140          | 0.020          | 0.000           | 0.010          | 0.010           | N                                     | None                 | —                        | Formed                   | 1.72 | Standard        |
| 35         | 0.300                                                             | 0.140          | 0.020          | 0.000           | 0.010          | 0.010           | Y                                     | Formed               | 2.25                     | Formed                   | 1.74 | VG              |
| 36X        | 0.300                                                             | 0.110          | 0.000          | 0.100           | 0.010          | 0.010           | N                                     | None                 | —                        | Formed                   | 1.55 | Standard        |
| 37         | 0.300                                                             | 0.110          | 0.000          | 0.100           | 0.010          | 0.010           | Y                                     | Formed               | 2.44                     | Formed                   | 1.58 | VG              |
| 38X        | 0.300                                                             | 0.110          | 0.000          | 0.030           | 0.000          | 0.010           | N                                     | None                 | —                        | Formed                   | 1.73 | Standard        |
| 39         | 0.300                                                             | 0.110          | 0.000          | 0.030           | 0.000          | 0.010           | Y                                     | Formed               | 2.18                     | Formed                   | 1.74 | VG              |
| 40X        | 0.300                                                             | 0.110          | 0.000          | 0.030           | 0.050          | 0.010           | N                                     | None                 | —                        | Formed                   | 1.53 | Standard        |
| 41         | 0.300                                                             | 0.110          | 0.000          | 0.030           | 0.050          | 0.010           | Y                                     | Formed               | 2.47                     | Formed                   | 1.55 | VG              |
| 42X        | 0.300                                                             | 0.110          | 0.000          | 0.030           | 0.010          | 0.000           | N                                     | None                 | —                        | Formed                   | 1.79 | Standard        |
| 43         | 0.300                                                             | 0.110          | 0.000          | 0.030           | 0.010          | 0.000           | Y                                     | Formed               | 2.23                     | Formed                   | 1.81 | VG              |
| 44X        | 0.300                                                             | 0.110          | 0.000          | 0.030           | 0.010          | 0.040           | N                                     | None                 | —                        | Formed                   | 1.66 | Standard        |
| 45         | 0.300                                                             | 0.110          | 0.000          | 0.030           | 0.010          | 0.040           | Y                                     | Formed               | 2.31                     | Formed                   | 1.67 | VG              |

TABLE 4

| Sample No. | Alloy composition:                                                                 |                 |               |           |               |            | Analysis results of surface structure |                      |                 | Saturation |               |
|------------|------------------------------------------------------------------------------------|-----------------|---------------|-----------|---------------|------------|---------------------------------------|----------------------|-----------------|------------|---------------|
|            | $(Fe_{(1-\alpha)}Co_{\alpha}Ni_{\beta})_{0.840}B_{0.11}Si_{0.03}C_{0.01}Cr_{0.01}$ |                 |               |           |               |            | Heat                                  | Co concentrated area |                 | SB         | magnetic flux |
|            | $(\gamma = 0, b = 0)$                                                              |                 |               | treated   |               |            |                                       | Co                   | concentrated    |            |               |
|            | Co <sub>α</sub>                                                                    | Ni <sub>β</sub> | or not Y or N | Formation | concentration | degree (-) | area Formation                        | Bs T                 | test Evaluation |            |               |
| 46X        | 0.300                                                                              | 0.005           | N             | None      | —             | —          | Formed                                | 1.74                 | Standard        |            |               |
| 47         | 0.300                                                                              | 0.005           | Y             | Formed    | 2.03          | —          | Formed                                | 1.75                 | VG              |            |               |

TABLE 4-continued

| Sample No.  | Alloy composition:                                                                    |               |           | Heat                     | Analysis results of surface structure |           | Saturation magnetic flux |               |
|-------------|---------------------------------------------------------------------------------------|---------------|-----------|--------------------------|---------------------------------------|-----------|--------------------------|---------------|
|             | $(Fe_{(1-\alpha+\beta)}Co_\alpha Ni_\beta)_{0.840}B_{0.11}Si_{0.03}C_{0.01}Cr_{0.01}$ |               |           |                          | Co concentrated area                  |           | SB                       | magnetic flux |
|             | $(\gamma = 0, b = 0)$                                                                 | treated       | Co        | concentrated             | density                               | Immersion |                          |               |
| Co $\alpha$ | Ni $\beta$                                                                            | or not Y or N | Formation | concentration degree (-) | area Formation                        | Bs T      | test Evaluation          |               |
| 48X-49      | 0.300                                                                                 | 0.200         | N         | None                     | —                                     | Formed    | 1.56                     | Standard      |
|             | 0.300                                                                                 | 0.200         | Y         | Formed                   | 1.34                                  | Formed    | 1.58                     | VG            |

TABLE 5

| Sample No.  | Alloy composition:                                                                           |          |               | Heat      | Analysis results of surface structure |                | Saturation magnetic |                 |
|-------------|----------------------------------------------------------------------------------------------|----------|---------------|-----------|---------------------------------------|----------------|---------------------|-----------------|
|             | $((Fe_{(1-\alpha)}Co_\alpha)_{1-\gamma}X1_\gamma)_{0.840}B_{0.11}Si_{0.03}C_{0.01}Cr_{0.01}$ |          |               |           | Co concentrated area                  |                | SB                  | flux            |
|             | $(\beta = 0, b = 0)$                                                                         | X1       | treated       | Co        | concentrated                          | density        |                     |                 |
| Co $\alpha$ | Element type                                                                                 | $\gamma$ | or not Y or N | Formation | concentration degree (-)              | area Formation | Bs T                | test Evaluation |
| 50X-51      | 0.300                                                                                        | Al       | 0.025         | N         | None                                  | —              | Formed              | 1.70            |
|             | 0.300                                                                                        | Al       | 0.025         | Y         | Formed                                | 2.29           | Formed              | 1.72            |
| 52X-53      | 0.300                                                                                        | Zn       | 0.025         | N         | None                                  | —              | Formed              | 1.70            |
|             | 0.300                                                                                        | Zn       | 0.025         | Y         | Formed                                | 2.24           | Formed              | 1.72            |
| 54X-55      | 0.300                                                                                        | Sn       | 0.025         | N         | None                                  | —              | Formed              | 1.69            |
|             | 0.300                                                                                        | Sn       | 0.025         | Y         | Formed                                | 2.25           | Formed              | 1.71            |
| 56X-57      | 0.300                                                                                        | Cu       | 0.025         | N         | None                                  | —              | Formed              | 1.68            |
|             | 0.300                                                                                        | Cu       | 0.025         | Y         | Formed                                | 2.28           | Formed              | 1.70            |
| 58X-59      | 0.300                                                                                        | Bi       | 0.025         | N         | None                                  | —              | Formed              | 1.69            |
|             | 0.300                                                                                        | Bi       | 0.025         | Y         | Formed                                | 2.32           | Formed              | 1.71            |
| 60X-61      | 0.300                                                                                        | La       | 0.025         | N         | None                                  | —              | Formed              | 1.59            |
|             | 0.300                                                                                        | La       | 0.025         | Y         | Formed                                | 2.22           | Formed              | 1.61            |
| 62X-63      | 0.300                                                                                        | Y        | 0.025         | N         | None                                  | —              | Formed              | 1.64            |
|             | 0.300                                                                                        | Y        | 0.025         | Y         | Formed                                | 2.25           | Formed              | 1.66            |
| 64X-65      | 0.300                                                                                        | Ga       | 0.025         | N         | None                                  | —              | Formed              | 1.64            |
|             | 0.300                                                                                        | Ga       | 0.025         | Y         | Formed                                | 2.28           | Formed              | 1.66            |
| 66X-67      | 0.300                                                                                        | Ti       | 0.025         | N         | None                                  | —              | Formed              | 1.59            |
|             | 0.300                                                                                        | Ti       | 0.025         | Y         | Formed                                | 2.31           | Formed              | 1.61            |
| 68X-69      | 0.300                                                                                        | Zr       | 0.025         | N         | None                                  | —              | Formed              | 1.60            |
|             | 0.300                                                                                        | Zr       | 0.025         | Y         | Formed                                | 2.29           | Formed              | 1.62            |
| 70X-71      | 0.300                                                                                        | Hf       | 0.025         | N         | None                                  | —              | Formed              | 1.59            |
|             | 0.300                                                                                        | Hf       | 0.025         | Y         | Formed                                | 2.24           | Formed              | 1.61            |
| 72X-73      | 0.300                                                                                        | Nb       | 0.025         | N         | None                                  | —              | Formed              | 1.59            |
|             | 0.300                                                                                        | Nb       | 0.025         | Y         | Formed                                | 2.26           | Formed              | 1.61            |

TABLE 6

| Sample No.  | Alloy composition:                                                                           |          |               | Heat      | Analysis results of surface structure |                | Saturation magnetic |                 |
|-------------|----------------------------------------------------------------------------------------------|----------|---------------|-----------|---------------------------------------|----------------|---------------------|-----------------|
|             | $((Fe_{(1-\alpha)}Co_\alpha)_{1-\gamma}X1_\gamma)_{0.840}B_{0.11}Si_{0.03}C_{0.01}Cr_{0.01}$ |          |               |           | Co concentrated area                  |                | SB                  | flux            |
|             | $(\beta = 0, b = 0)$                                                                         | X1       | treated       | Co        | concentrated                          | density        |                     |                 |
| Co $\alpha$ | Element type                                                                                 | $\gamma$ | or not Y or N | Formation | concentration degree (-)              | area Formation | Bs T                | test Evaluation |
| 74X-75      | 0.300                                                                                        | Ta       | 0.025         | N         | None                                  | —              | Formed              | 1.59            |
|             | 0.300                                                                                        | Ta       | 0.025         | Y         | Formed                                | 2.22           | Formed              | 1.61            |
| 76X-77      | 0.300                                                                                        | Mo       | 0.025         | N         | None                                  | —              | Formed              | 1.59            |
|             | 0.300                                                                                        | Mo       | 0.025         | Y         | Formed                                | 2.22           | Formed              | 1.61            |
| 78X-79      | 0.300                                                                                        | V        | 0.025         | N         | None                                  | —              | Formed              | 1.59            |
|             | 0.300                                                                                        | V        | 0.025         | Y         | Formed                                | 2.31           | Formed              | 1.61            |
| 80X-81      | 0.300                                                                                        | W        | 0.025         | N         | None                                  | —              | Formed              | 1.59            |
|             | 0.300                                                                                        | W        | 0.025         | Y         | Formed                                | 2.30           | Formed              | 1.61            |

TABLE 6-continued

| Alloy composition: $((Fe_{(1-\alpha)}Co_{\alpha})_{1-\gamma}X1_{\gamma})_{0.840}B_{0.11}Si_{0.03}C_{0.01}Cr_{0.01}$ |             |                |               |              |                      |                          | Analysis results of surface structure |                | Saturation magnetic flux |                 |
|---------------------------------------------------------------------------------------------------------------------|-------------|----------------|---------------|--------------|----------------------|--------------------------|---------------------------------------|----------------|--------------------------|-----------------|
| Sample No.                                                                                                          | Co $\alpha$ | (B = 0, b = 0) |               | Heat treated | Co concentrated area |                          | SB concentrated                       | area Formation | Bs density T             | test Evaluation |
|                                                                                                                     |             | X1             | or not Y or N |              | Formation            | concentration degree (-) |                                       |                |                          |                 |
| 82X                                                                                                                 | 0.300       | Ca             | 0.025         | N            | None                 | —                        | Formed                                | 1.67           | Standard                 |                 |
| 83                                                                                                                  | 0.300       | Ca             | 0.025         | Y            | Formed               | 2.22                     | Formed                                | 1.69           | VG                       |                 |
| 84X                                                                                                                 | 0.300       | Mg             | 0.025         | N            | None                 | —                        | Formed                                | 1.66           | Standard                 |                 |
| 85                                                                                                                  | 0.300       | Mg             | 0.025         | Y            | Formed               | 2.32                     | Formed                                | 1.68           | VG                       |                 |
| 86X                                                                                                                 | 0.300       | S              | 0.025         | N            | None                 | —                        | Formed                                | 1.68           | Standard                 |                 |
| 87                                                                                                                  | 0.300       | S              | 0.025         | Y            | Formed               | 2.24                     | Formed                                | 1.70           | VG                       |                 |
| 88X                                                                                                                 | 0.300       | N              | 0.025         | N            | None                 | —                        | Formed                                | 1.68           | Standard                 |                 |
| 89                                                                                                                  | 0.300       | N              | 0.025         | Y            | Formed               | 2.27                     | Formed                                | 1.70           | VG                       |                 |
| 90X                                                                                                                 | 0.300       | O              | 0.025         | N            | None                 | —                        | Formed                                | 1.68           | Standard                 |                 |
| 91                                                                                                                  | 0.300       | O              | 0.025         | Y            | Formed               | 2.12                     | Formed                                | 1.70           | VG                       |                 |

20

TABLE 7

| Alloy composition: $((Fe_{(1-\alpha)}Co_{\alpha})_{1-\gamma}X1_{\gamma})_{0.840}B_{0.11}Si_{0.03}C_{0.01}Cr_{0.01}$ |             |                |               |              |                      |                          | Analysis results of surface structure |                | Saturation magnetic |                 |
|---------------------------------------------------------------------------------------------------------------------|-------------|----------------|---------------|--------------|----------------------|--------------------------|---------------------------------------|----------------|---------------------|-----------------|
| Sample No.                                                                                                          | Co $\alpha$ | (B = 0, b = 0) |               | Heat treated | Co concentrated area |                          | SB concentrated                       | area Formation | Bs density T        | test Evaluation |
|                                                                                                                     |             | X1             | or not Y or N |              | Formation            | concentration degree (-) |                                       |                |                     |                 |
| 92X                                                                                                                 | 0.300       | Ag             | 0.025         | N            | None                 | —                        | Formed                                | 1.62           | Standard            |                 |
| 93                                                                                                                  | 0.300       | Ag             | 0.025         | Y            | Formed               | 2.29                     | Formed                                | 1.64           | VG                  |                 |
| 94X                                                                                                                 | 0.300       | As             | 0.025         | N            | None                 | —                        | Formed                                | 1.61           | Standard            |                 |
| 95                                                                                                                  | 0.300       | As             | 0.025         | Y            | Formed               | 2.32                     | Formed                                | 1.63           | VG                  |                 |
| 96X                                                                                                                 | 0.300       | Sb             | 0.025         | N            | None                 | —                        | Formed                                | 1.60           | Standard            |                 |
| 97                                                                                                                  | 0.300       | Sb             | 0.025         | Y            | Formed               | 2.27                     | Formed                                | 1.62           | VG                  |                 |
| 98X                                                                                                                 | 0.300       | Au             | 0.025         | N            | None                 | —                        | Formed                                | 1.62           | Standard            |                 |
| 99                                                                                                                  | 0.300       | Au             | 0.025         | Y            | Formed               | 2.25                     | Formed                                | 1.64           | VG                  |                 |
| 100X                                                                                                                | 0.300       | Pt             | 0.025         | N            | None                 | —                        | Formed                                | 1.60           | Standard            |                 |
| 101                                                                                                                 | 0.300       | Pt             | 0.025         | Y            | Formed               | 2.26                     | Formed                                | 1.62           | VG                  |                 |

As shown in Table 2 to Table 7, in the sample which was performed with the predetermined heat treatment exhibited a higher corrosion resistance than the sample without the heat treatment. Thus, from this result, within the alloy composition range shown in Experiment 2, by forming the Co concentrated area 11 and the SB concentrated area 12, the corrosion resistance was improved while maintaining a high Bs.

Note that, according to the results shown in Table 2, as the Co amount increased in the internal area 2 (that is, as the Co amount of the soft magnetic alloy increased), it took longer time till the rust was formed (longer rust formation time). That is, as the Co amount in the internal area 2 increased, the corrosion resistance which is an absolute evaluation improved. Note that, as Sample No. 25 of Table 2 shows, when the Co amount in the internal area 2 was high, the Co concentration degree rather tended to decrease. Also, compared to Sample No. 25, a relative improvement effect of the corrosion resistance (that is, the corrosion resistance with respect to the standard alloy) was better in Sample No. 13, 15, 17, 19, 21, and 23 which had high Co concentration degree. That is, according to this result, as the Co concentration degree increased, the improvement effect of the corrosion resistance with respect to the standard alloy (the

sample without the heat treatment which was the treatment for forming the concentrated area) was further enhanced.

### Experiment 3

In Experiment 3, an amorphous soft magnetic alloy powder having the amorphous degree X of 85% or more (Sample No. 1 and 5), and a nanocrystal soft magnetic alloy powder having the amorphous degree X of less than 85% (Sample No. 102 and 103), and a crystalline soft magnetic alloy powder having the amorphous degree X of less than 85% (Sample No. 104 and 105) were produced. Then, the influence to the corrosion resistance due to the difference in the crystal structures of the soft magnetic alloys was examined.

In Experiment 3, the crystal structure of each sample was regulated by a pre-heat treatment. Specifically, in Sample No. 1 and 5 of Experiment 3, an amorphous soft magnetic alloy powder was obtained since the pre-heat treatment was not performed. Also, in Sample No. 102 and 103 of Experiment 3, by performing the pre-heat treatment at a holding temperature: 500° C. for a holding time: 10 min, a nanocrystal soft magnetic alloy powder was obtained. Also, in Sample No. 104 and 105 of Experiment 3, by performing the pre-heat treatment at a holding temperature: 650° C. for a holding time: 1 hour, a crystalline soft magnetic alloy

powder was obtained. Note that, other conditions of the above-mentioned pre-heat treatment were, a temperature increasing rate: 100° C./min, a furnace atmosphere: Ar atmosphere, and a gauge pressure inside the heating furnace: 0.0 kPa, thereby the crystal structure was controlled in a state which did not form the Co concentrated area.

The composition of the soft magnetic alloy of each sample of Experiment 3 was  $(Fe_{0.7}Co_{0.3})_{0.84}B_{0.11}Si_{0.03}C_{0.01}Cr_{0.01}$ . Also, in Experiment 3, for each crystal structure, a sample carried out with the heat treatment for forming each concentrated area (11 and 12), and a sample without the heat treatment were produced. In Table 8, the sample performed with the heat treatment was shown as "Y", and the sample without the heat treatment was shown as "N". Note that, for samples which were performed with the pre-heat treatment (Sample No. 103 and 105), the heat treatment for forming each concentrated area (11 and 12) was performed after the pre-heat treatment. Also, conditions of the heat treatment of Experiment 3 were a holding temperature: 200° C., a holding time: 1 h, an oxygen concentration in a heating furnace: 100 ppm, and a gauge pressure in the heating furnace: 0.3 kPa.

Also, in Experiment 3 as similar to Experiment 2, Bs was measured and the immersion test was performed. Regarding the immersion test of Experiment 3, for the same crystal structure, the rust formation time of a sample without the heat treat was defined as  $T_N$ , and the rust formation time of a sample performed with the heat treatment was defined as  $T_Y$ , then a sample which showed  $T_Y/T_N \leq 1.0$  was evaluated as "NG (Not Good)", a sample which showed  $1.0 < T_Y/T_N < 1.2$  was evaluated as "G (Good)", and a sample which showed  $1.2 \leq T_Y/T_N$  was evaluated "VG (Very Good)". Evaluation results are shown in Table 8.

phous, the improvement effect of the corrosion resistance was particularly good.

#### Experiment 4

In Experiment 4, the soft magnetic alloy samples of a ribbon form (Sample No. 106 and 107) were produced by using a single roll method. Conditions for forming a ribbon were, a temperature of a molten sprayed to a roll: 1300° C., a roll temperature: 30° C., and a roll rotation speed: 25 m/sec. Also, the inside of the chamber was air atmosphere. The soft magnetic alloy ribbon obtained under the above-mentioned conditions had a thickness of 20 to 25  $\mu$ m, a width of a short direction of about 5 mm, and a length of ribbon of about 10 m.

Also, in Experiment 4, as similar to Experiment 1, the alloy compositions of Sample No. 106 and 107 were measured using ICP, and it was confirmed that both samples satisfied the compositional formula:  $(Fe_{0.7}Co_{0.3})_{0.84}B_{0.11}Si_{0.03}C_{0.01}Cr_{0.01}$  (atomic ratios;  $\alpha=0.300$ ,  $\beta=0$ ,  $\gamma=0$ ,  $a=0.110$ ,  $b=0$ ,  $c=0.030$ ,  $d=0.010$ , and  $e=0.010$ ). Further, when the crystal structure of the soft magnetic alloy ribbons of Sample No. 106 and 107 were measured using XRD, the amorphous crystal structure having the amorphous degree X: 85% or higher was confirmed in both of Sample No. 106 and 107.

For the soft magnetic alloy ribbon of Sample No. 106, the heat treatment was not performed, and an analysis of the surface structure, Bs measurement, and the immersion test were performed. On the other hand, the soft magnetic alloy ribbon of Sample No. 107 was performed with a heat treatment under the conditions shown in Table 9, and the same evaluations as for Sample No. 106 were carried out. Note that, in the immersion test of the soft magnetic alloy

TABLE 8

| Sample No. | Alloy composition:                                                |      |     |      |      |      |             | oxidizing treatment at low temp) | 熱処理    | Analysis results of surface structure |           |                | Saturation magnetic flux |                 |  |  |
|------------|-------------------------------------------------------------------|------|-----|------|------|------|-------------|----------------------------------|--------|---------------------------------------|-----------|----------------|--------------------------|-----------------|--|--|
|            | $(Fe_{(1-\alpha)}Co_{\alpha})_{(1-(a+b+c+d+e))}B_aP_bSi_cC_dCr_e$ |      |     |      |      |      |             |                                  |        | Co concentrated area                  |           |                | SB                       | flux            |  |  |
|            | $(\beta = 0, \gamma = 0)$                                         |      |     |      |      |      |             |                                  |        | Formation                             |           |                | concentrated             | density         |  |  |
|            | Co $\alpha$                                                       | B a  | P b | Si c | C d  | Cr e | Formation   |                                  |        | area Formation                        | Formation | area Formation | Bs T                     | test Evaluation |  |  |
| 1-X        | 0.30                                                              | 0.11 | 0   | 0.03 | 0.01 | 0.01 | Amorphous   | N                                | None   | —                                     | Formed    | 1.73           | Standard                 |                 |  |  |
| 5          | 0.30                                                              | 0.11 | 0   | 0.03 | 0.01 | 0.01 | Amorphous   | Y                                | Formed | 1.91                                  | Formed    | 1.75           | VG                       |                 |  |  |
| 102-X      | 0.30                                                              | 0.11 | 0   | 0.03 | 0.01 | 0.01 | Nanocrystal | N                                | None   | —                                     | Formed    | 1.75           | Standard                 |                 |  |  |
| 103        | 0.30                                                              | 0.11 | 0   | 0.03 | 0.01 | 0.01 | Nanocrystal | Y                                | Formed | 1.87                                  | Formed    | 1.75           | VG                       |                 |  |  |
| 104-X      | 0.30                                                              | 0.11 | 0   | 0.03 | 0.01 | 0.01 | Crystalline | N                                | None   | —                                     | Formed    | 1.83           | Standard                 |                 |  |  |
| 105        | 0.30                                                              | 0.11 | 0   | 0.03 | 0.01 | 0.01 | Crystalline | Y                                | Formed | 1.75                                  | Formed    | 1.83           | VG                       |                 |  |  |

Table 8 shows that, as similar to the amorphous soft magnetic alloy, in the nanocrystal or crystalline soft magnetic alloy, Sample No. 103 and 105 which were formed with the Co concentrated area 11 and the SB concentrated area 12 by performing the predetermined heat treatment showed improved corrosion resistance compared to Sample No. 102 and 104 which were not heat treated. Also, by comparing the results of Sample No. 102 to 105 shown in Table 8 and the results of Sample No. 1 and 5, it can be understood that when the soft magnetic alloy was am-

ribbon, the ribbon was cut into an arbitrary size (a length of about 4 cm×a width of about 5 mm) to prepare a sample for immersion test. Then, the sample of a ribbon form for immersion test was immersed in tap water. Results of the immersion test of Experiment 4 were evaluated as same as Experiment 1. The evaluation result of each sample of Experiment 4 is shown in Table 9. Note that, Table 9 includes the experiment results of the soft magnetic alloy powders (Sample No. 1 and 5 of Experiment 1) having the same alloy composition as Sample No. 106 and 107.

TABLE 9

| Sample No. | Form of soft magnetic alloy | Analysis results of surface structure |                |                          |                      |           |                                | Saturation                 |                           |
|------------|-----------------------------|---------------------------------------|----------------|--------------------------|----------------------|-----------|--------------------------------|----------------------------|---------------------------|
|            |                             | He treatment condition                |                |                          | Co concentrated area |           | SB concentrated area Formation | magnetic flux density Bs T | Immersion test Evaluation |
|            |                             | Holding Temp. °C.                     | Holding time h | Oxygen concentration ppm | Gauge pressure kPa   | Formation |                                |                            |                           |
| 1X         | Powder                      | —                                     | —              | —                        | —                    | None      | —                              | Formed                     | 1.73 Standard             |
| 5          | Powder                      | 200                                   | 1.0            | 100                      | 0.30                 | Formed    | 1.91                           | Formed                     | 1.75 VG                   |
| 106X       | Ribbon                      | —                                     | —              | —                        | —                    | None      | —                              | Formed                     | 1.73 Standard             |
| 107        | Ribbon                      | 200                                   | 1.0            | 100                      | 0.30                 | Formed    | 1.88                           | Formed                     | 1.75 VG                   |

As shown in Table 9, when the soft magnetic alloy was a ribbon form, by forming the Co concentrated area **11** and the SB concentrated area **12** by performing the predetermined heat treatment, the corrosion resistance can be improved while maintaining a high Bs.

## NUMERICAL REFERENCES

- 1, 1a, 1b . . .** Soft magnetic alloy  
**2 . . .** Internal area  
**10 . . .** Outermost surface  
**11 . . .** Co concentrated area  
**12 . . .** SB concentrated area  
**13 . . .** Oxide layer  
**20 . . .** Coating layer

What is claimed is:

- 1.** A soft magnetic alloy comprising  
 an internal area having a soft magnetic alloy composition  
 including Fe and Co,  
 a Co concentrated area existing closer to a surface side  
 than the internal area and having a higher Co concen-  
 tration than in the internal area, and  
 a Si and/or B concentrated area existing closer to the  
 surface side than the Co concentrated area and having  
 a higher concentration of at least one element selected  
 from Si and B than in the internal area, wherein  
 the Co concentrated area is a metal phase.  
**2.** The soft magnetic alloy according to claim **1**, wherein  
 the Si and/or B concentrated area comprises an oxide phase.  
**3.** The soft magnetic alloy according to claim **1**, wherein  
 the Si and/or B concentrated area comprises an amorphous  
 structure.

15      4. The soft magnetic metal according to claim **1**, wherein  
 a Co concentration degree in the Co concentrated area is  
 larger than 1.2.

5      5. The soft magnetic alloy according to claim **1** having an  
 amorphous degree of 85% or more.

20      6. The soft magnetic alloy according to claim **1** being a  
 ribbon form.

7. The soft magnetic alloy according to claim **1** being a  
 powder form.

8. A magnetic component including the soft magnetic  
 alloy according to claim **1**.

25      9. The soft magnetic metal according to claim **1**, wherein  
 the soft magnetic alloy composition has a compositional  
 formula of  $(Fe_{(1-\alpha-\beta)}Co_{\alpha}Ni_{\beta})_{1-\gamma}X_{1-\gamma}(1-(a+b+c+d+e))B_aP_b-$   
 $Si_cC_dCr_e$ , wherein X1 is at least one selected from the group  
 consisting of Ti, Zr, Hf, Nb, Ta, Mo, W, Al, Ga, Ag, Zn, S,  
 30 Ca, Mg, V, Sn, As, Sb, Bi, N, O, Au, Cu, rare earth elements,  
 and platinum group elements,  $0.005 \leq \alpha \leq 0.700$ ,  $0 \leq \beta \leq 0.200$ ,  
 $0 \leq \gamma \leq 0.030$ ,  $0 \leq a \leq 0.200$ ,  $0 \leq b \leq 0.100$ ,  $0 \leq c \leq 0.150$ ,  $0 \leq d \leq 0.050$   
 and  $0 \leq e \leq 0.050$ .

35      10. The soft magnetic metal according to claim **9**, wherein  
 $0.050 \leq \alpha \leq 0.600$ ,  $0.005 \leq \beta \leq 0.010$ ,  $0 \leq a \leq 0.150$ ,  
 $0.005 \leq b \leq 0.050$ ,  $0.001 \leq c \leq 0.070$ ,  $0 \leq d \leq 0.020$  and  
 $0.001 \leq e \leq 0.020$ .

40      11. The soft magnetic metal according to claim **1**, wherein  
 when a sum of atomic ratios of elements constituting the soft  
 magnetic alloy is 1, an atomic ratio of a total amount of Fe,  
 Co, Ni, and X1 is within a range of  $0.720 \leq (1-(a+b+c+d+e)) \leq 0.950$ .

12. The soft magnetic metal according to claim **11**,  
 wherein the range is  $0.780 \leq (1-(a+b+c+d+e)) \leq 0.890$ .

45      13. The soft magnetic metal according to claim **11**,  
 wherein the range is  $0.720 \leq (1-(a+b+c+d+e)) \leq 0.890$ .

\* \* \* \* \*